# EUROPEAN PATENT SPECIFICATION

(11) **EP 3 341 513 B1**
(45) Date of publication and mention of the grant of the patent: **24.11.2021**
(21) Application number: 16760310.9
(22) Date of filing: 26.08.2016
(51) Int. Cl.: D04H 1/4374, A44B 18/00, D04H 1/54, D04H 1/559, D04H 11/08

(54) **LOOP MEMBER FOR SURFACE FASTENER AND ADULT DIAPER**
SCHLAUFENELEMENT FÜR OBERFLÄCHENVERSCHLUSS UND WINDEL FÜR ERWACHSENE
ÉLÉMENT FORMANT BOUCLE POUR DISPOSITIF DE FIXATION DE SURFACE ET COUCHE POUR ADULTE

(30) Priority: 28.08.2015 JP 2015169458
(43) Date of publication of application: 04.07.2018
(73) Proprietor: 3M Innovative Properties Company, St. Paul, MN 55133-3427 (US)
(72) Inventor: MORISHITA, Kenichiro, Shinagawa-ku Tokyo 141-8684 (JP)
(74) Representative: Vossius & Partner Patentanwälte Rechtsanwälte mbB
(86) International application number: PCT/US2016/048860
(87) International publication number: WO 2017/040240

(56) References cited:
- EP-A1- 0 765 616
- EP-A1- 1 181 873
- WO-A1-2016/007431
- WO-A2-02/100207
- US-A1- 2008 260 989

## Description

### FIELD OF THE INVENTION

The present invention relates to a loop member for a surface fastener, and a diaper for adults.

### BACKGROUND TECHNOLOGY

Conventionally surface fasteners are widely used for fixing and securing various types of item such as fiber products, plastic products, paper products, industrial components, electronic components, building materials, and the like. For example, surface fasteners fitted to sanitary articles (for example, paper diapers and the like) as fastening members are known. Surface fasteners with various types of fastening configurations are known, for example, fasteners that include a pair of a male member having a hook-shaped engaging element and a female member that can be engaged with the engaging element, and the like. Among these, fastening members for surface fasteners using nonwoven fabrics have the advantage of excellent pliability and air permeability, so conventionally many types have been proposed.

WO 2008/130807 discloses a loop material for a hook and loop fastener made from a composite nonwoven fabric. The composite nonwoven fabric has a carded nonwoven fabric loop layer of thermoplastic crimped staple fiber, the staple fiber being 1.5 to 6.0 dTEX, the carded nonwoven fabric comprising a base material layer of a spunbond or spunmelt nonwoven fabric having an basis weight from 10 to 35 g/m²; and a plurality of substantially air impermeable bonding regions at which the loop layer is joined to the base material layer, the bonding regions including from 35 to 55% of the surface area of the loop material.

US 5,786,060 discloses a female member for a surface fastener that includes: a web which includes a thermal fusion bonded composite fiber body; a plurality of entangled loops formed on a first surface of the web; and a compressed thermal fusion bonded layer formed on a second surface of the web. By making the second surface denser than the first surface, the plurality of entangled loops formed in the first surface can be forcibly engaged with elements formed on the surface of a male member. The peeling strength necessary to separate the plurality of entangled loops from the elements formed on the surface of the male member is at least 20 gf/cm.

US 5,470,424 discloses a method of manufacturing a liquid impermeable and air permeable sheet having a fibrous surface. The method includes: forming a sheet having a first fibrous surface and a second fibrous surface; melting the fiber on the first surface without significantly altering the fiber of the second surface by subjecting the sheet to sufficient pressure and a Z gradient temperature differential to form a liquid impermeable and air impermeable skin from the melted material; depositing fiber on the skin while the skin is in at least a semi-melted state to form a fiber / skin / fiber material; and making the liquid impermeable and air impermeable skin air permeable while maintaining its liquid impermeability.

EP 1 181 873 A1 relates to a fastener which has a high engaging force, which generates fluffing only very slightly and which is prevented from being lowered in engaging force after repeated attachment and detachment. WO 2016/007431 A1 relates to a surface fastener loop member and a sanitary article.

### SUMMARY OF THE INVENTION

In the case of diapers for adults, for example, in some cases, the diaper is combined with a pad that is disposed therein, and a pattern of use is adopted in which the diaper is used for a comparatively long period of time by frequently changing the pad inside only, and replacing the outside diaper every three days, for example (or about once every 20 times that the pad is changed). In this case, it is required that the surface fastener of the diaper can maintain good engagement strength (in particular, peeling strength and shear strength) between the fastening members after many repetitions (for example, 20 repetitions) of fastening and unfastening of the pair of fastening members (in other words, durability of engagement strength under repeated fastening and unfastening). However, when the engaging element is a loop member that is a nonwoven fabric (in particular, a short fiber nonwoven fabric), the fiber from which the nonwoven fabric is constituted can easily be shed or be damaged due to repeated fastening and unfastening, and it is difficult to obtain durability of engagement strength under repeated fastening and unfastening. On the other hand in the case of for example knit loops, normally, the durability of engagement strength is good under repeated fastening and unfastening, but its air permeability and pliability are low. Therefore, it is desirable to have fastening members with excellent durability of engagement strength under repeated fastening and unfastening, while maintaining good air permeability and pliability by using nonwoven fabric.

Also, in articles having surface fasteners (for example, sanitary articles such as diapers), in some cases, a fastening member for a surface fastener having a printed layer is used. In one example of such a fastening member for a surface fastener, the printed layer is formed on one primary surface of a nonwoven fabric, and the other primary surface is used as the engagement surface with the other fastening member for a surface fastener, and pattern provided on the printed layer is visible through the nonwoven fabric. By fixing the primary surface on the printed layer side of the fastening member for a surface fastener to the body portion of an article, an article having a surface fastener with a pattern can be formed. However, the image sharpness of the printed layer provided on the nonwoven fabric is not necessarily sufficiently satisfactory. It is also desirable to further reduce the cost of fastening members.

In order to solve the above problems, it is an object of the present invention to provide a fastening member for a surface fastener, or more specifically a loop member, with good air permeability, pliability, engagement strength between the pair of fastening members, durability of engagement strength under repeated fastening and unfastening, and printing properties (image sharpness of the printed layer), and that can be manufactured at low cost.

The invention is defined by independent claim 1 and further embodiments are defined by the dependent claims. One aspect of the present invention provides a loop member for a surface fastener, comprising: a loop layer; and a base material layer, the loop layer including fusion bonded short fiber nonwoven fabric, the base material layer including calendered short fiber nonwoven fabric, the ratio of the average fineness of the fiber in the loop layer to the average fineness of the fiber in the base material layer [average fineness of fiber in loop layer / average fineness of fiber in base material layer] being from 2 to 18, and the thickness of the base material layer being from 15 µm to 100 µm, wherein the short fiber nonwoven fabric of the loop layer includes core-in-sheath fibers that include a polypropylene core with a first melting point, and a polyethylene sheath with a second melting point that is lower than the first melting point, and has an average fineness of 4.0 deniers or greater and 10.0 deniers or less, as measured by an average fineness measurement as described in the description.

Another aspect of the present invention provides an adult diaper that includes the above-described loop member.

### EFFECT OF THE INVENTION

According to the present invention, it is possible to provide a loop member for a surface fastener and an adult diaper with good air permeability, pliability, engagement strength, durability of engagement strength under repeated fastening and unfastening, and printing properties and that can be manufactured at low cost.

### BRIEF DESCRIPTION OF THE DRAWINGS

FIG. 1 illustrates an example of a loop member according to one aspect of the present invention.
FIG. 2 illustrates an example of a loop member according to one aspect of the present invention, showing the loop layer and the base material layer secured by embossing.
FIG. 3 illustrates an image of the surface of the loop layer in Working Example 1.
FIG. 4 illustrates an image of the surface of the loop layer in Comparative Example 1.

### BEST MODE FOR CARRYING OUT THE INVENTION

Exemplary embodiments of the present invention are described below, but the present invention is not restricted to the following embodiments, and any variation that does not violate the scope of the patent claims are intended to be included in the present invention. Note that unless otherwise noted, the various property values referred to in this disclosure are intended to be values measured by the methods disclosed in the [Examples] section, or by a method considered to be equivalent to these methods by one skilled in the art.

The present disclosure provides, a loop member for a surface fastener, comprising: a loop layer; and a base material layer, the loop layer including fusion bonded short fiber nonwoven fabric, the base material layer including calendered short fiber nonwoven fabric, the ratio of the average fineness of the fiber in the loop layer to the average fineness of the fiber in the base material layer [average fineness of fiber in loop layer / average fineness of the fiber in base material layer] being from 1.5 to 30, and the thickness of the base material layer being from 15 µm to 100 µm.

The loop member of the present disclosure can be used as a loop member forming a surface fastener by various conventional commonly known fastening means. In one aspect, the loop member according to the present disclosure can be used as a female member, to form a surface fastener in combination with a male member. In another aspect, a surface fastener may be a pair of members in which the structure of both a male member and a female member that is the loop member according to the present disclosure are disposed coplanarly. The loop member according to the present disclosure may be directly engaged with, for example, a wall, a cloth or the like.

More specifically, in the loop member of the present disclosure, the short fiber nonwoven fabric included in the loop layer functions as an engaging element, and the short fiber nonwoven fabric included in the base material layer is intended to form a printed surface. For example, hooks are desirable as male members from the point of view of being able to strongly engage with an engaging element that is a nonwoven fabric. Hooks are configured from projections that project in the thickness direction of the surface fastener. The type of projection does not matter provided the engaging force is satisfied, but, for example, mushroom-shaped, anchor-shaped, or J-shaped hooks are desirable. Normally, the pin density is from about 77.5 to 775 per square centimeter (500 to 5000 per square inch). The material can be selected from polypropylene, polyester, polyethylene, polyamide, and their copolymers and mixtures. The loop member according to the present disclosure may be a part of a fastening member configured from hooks, and a loop layer that includes short fiber nonwoven fabric as engaging element that can be engaged with the hooks, disposed coplanarly.

FIG. 1 illustrates an example of a loop member according to one aspect of the present invention. Referring to FIG. 1, a loop member 1 includes a base material layer 11 and a loop layer 12. In a typical aspect, the loop member 1 can further include a printed layer 13.

The loop layer and the base material layer include short fiber nonwoven fabric. In a typical aspect, the loop member can be substantially constituted from nonwoven fabric, and more typically can be substantially constituted from short fiber nonwoven fabric. A loop member substantially constituted from nonwoven fabric can have an appropriate amount of pliability and air permeability for use as a sanitary article. Short fiber nonwoven fabrics have the advantage that thin and pliable layers can be formed. Note that in the present disclosure, "short fiber nonwoven fabric" is intended to refer to nonwoven fabric that is at least mostly (50% or more of the mass of the constituent fiber) constituted from staple (in other words, short fibers), as distinct from nonwoven fabric constituted from filaments (in other words, long fibers). Short fiber nonwoven fabric includes carded nonwoven fabric, air-laid nonwoven fabric, wet-laid nonwoven fabric, and the like. On the other hand, long fiber nonwoven fabric normally includes spunbond nonwoven fabric and the like. Although not limited to this, staple normally has a fiber length of several hundreds of mm or less.

The loop layer includes fusion bonded short fiber nonwoven fabric. In the present disclosure, "fusion bonded short fiber nonwoven fabric" is intended to refer to short fiber nonwoven fabric having a form in which the fibers from which the short fiber nonwoven fabric is constituted are bonded together by fusion of the fiber. Fusion bonding of the short fiber nonwoven fabric can be confirmed by observation (for example, observation using an optical microscope) of traces of fusion of the fiber material on the fiber surface of the short fiber nonwoven fabric, and bonding of fibers together at the positions of these traces of fusion. Traces of fusion is intended to refer to traces of a process applied with the object of causing fusion bonding in the loop layer only (and therefore can only be seen in the loop layer), and for example is to be distinguished from traces of fusion produced by processes with other objects, such as joining the loop layer and the base material layer (these traces of fusion can be seen throughout both the loop layer and the base material layer), and the like. Also, fusion bonding can be confirmed by touching the short fiber nonwoven fabric with the hand and observing that the surface has become comparatively stiffer. In the present disclosure, the fusion bonding to form the fusion bonded short fiber nonwoven fabric can be obtained by, for example, forming with a high temperature air-through process. In the present disclosure, "high temperature air-through process" is intended to refer to a process that passes air at high temperature (at or above the melting point of the material of the outside of the fiber of the short fiber nonwoven fabric) through the thickness direction of the short fiber nonwoven fabric. Other methods of fusion bonding that can be considered include means for heating at a high temperature without passing air through, or causing fusion of the outside of the fibers with chemicals to produce bonds between fibers. However, high temperature air-through processing is desirable from the point of view of causing fusion bonding not only on the surface of the short fiber nonwoven fabric, but also on the (outside of the fibers on the) interior thereof. Also, high temperature air-through processing is preferable since the chemicals used for fusion of the fibers are often kept at a distance in an application of a sanitary article such as a diaper or the like. By fusion bonding the fibers not by a method that directly applies large pressure to the short fiber nonwoven fabric with a roll or the like, the durability of the loop member can be increased while maintaining the engaging force.

The base material layer includes calendered short fiber nonwoven fabric. In the present disclosure, "calendered short fiber nonwoven fabric" refers to short fiber nonwoven fabric having a surface condition that has been smoothed by the application of pressure. Therefore, in the present disclosure, in addition to passing the layer to be processed between a pair of smooth rolls with the purpose of smoothing the layer, the calendering to form calendered short fiber nonwoven fabric includes, for example, processes to smooth the layer to be processed by passing the layer to be processed between a smooth roll and an uneven roll (for example, a thermal bond roll). Note that when for example an uneven roll is used, adjusting the process to obtain the required smoothing effect (for example, carrying out the operation of passing the layer to be processed between the rolls several times, adjusting the point bond conditions so that the processed area is comparatively large in the point bonding described later, and the like) can be carried out as appropriate by a person skilled in the art. Note that the "high temperature air-through process" and the "calendering" described above differ in that the latter is a process in which the short fiber nonwoven fabric directly contacts the rolls or the like with the purpose of smoothing, whereas the former is not.

In the loop member according to the present disclosure, the base material layer and the loop layer are separate layers, so the properties of each layer can each be controlled independently in accordance with the purpose. The inventors focused on the requirement for a printed surface with high smoothness in order to achieve good printing properties (in other words, achieving a printed design with image sharpness), and in addition focused on the requirement for ensuring the engagement strength (in particular the peeling strength and the shear strength) and the durability of engagement strength under repeated fastening and unfastening of a pair of fastening members (for example, a male member, referred to as hooks, when the loop member of the present disclosure is used as the female member). The inventors also focused on the main reasons that conventionally the printed image did not have image sharpness, namely the printed surface was not flat because the nonwoven fabric was point bonded and therefore the ink drops on the printed surface were not stable, and the loop member was thick, and the printed image appeared blurred when the printed layer was viewed through the loop member. In addition the inventors focused on the fact that conventional loop members using nonwoven fabric are not provided with durability of engagement strength to withstand repeated fastening and unfastening.

Then the inventors discovered that by laminating the loop layer that includes the nonwoven fabric that has a fineness that is larger than that of the nonwoven fabric used in the base material layer and is fusion bonded, and the base material layer that is made thin and smooth in the calendering, it was possible to achieve both engagement strength between the fastening members and durability of engagement strength under repeated fastening and unfastening, and a high level of printing properties and shape retaining properties as a member. Also, the thin loop member (in other words, the laminate of the loop layer and the base material layer) has the advantages of low cost and excellent pliability.

The loop layer functions as an engaging element. In one aspect, the short fiber nonwoven fabric included in the loop layer can engage with hooks. Note that various types of thermoplastic resin materials can be used as the material of the hooks, such as, for example, polyethylene (for example high density polyethylene), polypropylene, polystyrene, polyvinyl chloride, polyethylene terephthalate, polybutylene terephthalate, nylon, polycarbonate, polymethyl methacrylate, polyacetal, polymethyl pentene, acrylonitrile-styrene-butadiene, polyphenylene ether, polyphenylene sulfide, as well as styrene-based elastomers such as styrene-butadiene-styrene, styrene-isoprene-styrene and the like, olefin-based elastomers such as ethylene-α-olefin copolymer and the like, ester-based elastomers, amide-based elastomers, urethane-based elastomers, vinyl chloride-based elastomers, silicone-based elastomers, fluorine-based elastomers, and their alloys, and the like.

The fiber from which the short fiber nonwoven fabric included in the loop layer and the base material layer are constituted can be polyolefin (for example polyethylene, polypropylene, and the like), polyester (for example, PET, PBT, and the like), polyamide, polyurethane, EVA (ethylene vinyl acetate), polylactate, rayon, their copolymers and mixtures, as well as natural fibers, and the like.

In one aspect, high strength polyamide can be used in the loop layer from the point of view of preventing loop layer breakage (pull out of the fibers, and the like) due to engaging with another fastening member. On the other hand, taking material cost and environmental stability into consideration, polyethylene, polypropylene, polyester, or the like can be used in the loop layer and/or the base material layer.

The fibers constituting the short fiber nonwoven fabric may be hydrophilic or hydrophobic. The fibers may also be composite fibers. Examples of preferable fiber forms of the composite fiber include core-in-sheath types (concentric types and eccentric types), parallel types (i.e., side-by-side types), and split types (for example the fiber cross-section is split into arc forms). Also the fiber may be deformed cross-section fiber, crimped fiber, thermal contraction fiber, and the like. These fibers may be used singly or in combinations of two or more kinds.

A two-component-type elastic composite fiber having a hard elastic component including crystalline polypropylene as a first component and having a thermoplastic elastomer as a second component, or a blended fiber that combines this with another fiber can be used.

In a preferred aspect, the fiber from which the short fiber nonwoven fabric included in the loop layer is constituted has a core-in-sheath structure. Also, in a preferred aspect, the fiber from which the short fiber nonwoven fabric included in both the loop layer and the base material layer is constituted has a core-in-sheath structure. A fiber having a core-in-sheath structure has a core with a first melting point (for example, polyamide), and a sheath with a second melting point that is lower than the first melting point (for example, polyethylene), and has the advantage of excellent thermal fusion bonding properties. Taking material cost and environmental stability into consideration, and that preferably polyethylene, polypropylene, polyester, or the like are used in the loop layer and/or the base material layer, examples of core-in-sheath fiber having a core with a first melting point and a sheath with a second melting point that is lower than the first melting point include a core-in-sheath fiber having a polypropylene core and a polyethylene sheath, a core-in-sheath fiber having a polypropylene core and a modified polyethylene sheath, a core-in-sheath fiber having a polypropylene core and a modified polypropylene sheath, and the like. In one aspect, a core-in-sheath fiber having a polypropylene core and a polyethylene sheath can be selected from the point of view of light weight, high strength, high pliability, and the like. In particular, including short fiber nonwoven fabric constituted from fiber having the core-in-sheath structure as described above is advantageous from the point of view of forming the fusion bonded sites well.

For example, in a preferred aspect in which the fiber from which the short fiber nonwoven fabric included in the loop layer is constituted is core-in-sheath fiber having a core with a first melting point and a sheath with a second melting point, the first melting point is about 150°C or higher, or about 160°C or higher, or about 170°C or higher, from the point of view of obtaining good mechanical strength for the loop layer. If polyethylene or polypropylene is used, from the material properties, the first melting point will be about 200°C or less, and if polyester is used, from the material properties, the first melting point will be about 300°C or less. Also, in a preferred aspect, the second melting point is about 130°C or less, or about 120°C or less, or about 110°C or less, from the point of view of obtaining good mechanical strength of the loop layer, from the point of view of forming the fixing sites of the loop layer well by fusion bonding, and from the point of view of obtaining good pliability of the loop layer, and is about 80°C or more or about 100°C or more from the point of view of using a polymer material. Combining the first melting point in the range as described above and the second melting point in the range as described above is particularly preferable. Note that the first melting point in the range as described above and the second melting point in the range as described above and their combination are also advantageous in the base material layer from the point of view of forming short fiber nonwoven fabric with excellent air permeability and smoothness. Note that if the core has a plurality of melting points and if the sheath has a plurality of melting points, these properties can also be obtained. In this case, any of the plurality of melting points of the core are the first melting point, any of the plurality of melting points of the sheath are the second melting point, and in particular the lowest of each contributes to the fusion bonding and shape retention. In one aspect, the first melting point of the core and the second melting point of the sheath in the present disclosure may be the lowest first melting point of the core and the lowest second melting point of the sheath respectively. Note that the melting point is the value measured by DSC or the like.

In another preferred aspect, the fiber from which the short fiber nonwoven fabric included in the loop layer may be, for example, fiber of a single material having a melting point in the range given above for the first melting point.

In a preferred aspect, the average fineness of the loop layer is about 2.0 deniers or more and about 15 deniers or less. From the point of view of obtaining good engagement strength preferably the average fineness is about 2.0 deniers or more, or about 4.0 deniers or more, and from the point of view of maintaining good pliability of the loop member preferably the average fineness is about 15.0 deniers or less, or about 12.0 deniers or less, or about 10.0 deniers or less, or about 8.0 deniers or less, or about 6.0 deniers or less.

In a preferred aspect, the average fineness of the base material layer is about 0.5 deniers or more and about 3.0 deniers or less. From the point of view of maintaining the mechanical strength and ease of manufacture of the base material layer, preferably the average fineness is about 0.5 deniers or more, or about 0.7 deniers or more, or about 0.9 deniers or more, or about 1.0 deniers or more. From the point of view of applying a smooth printing surface and contributing to good printing properties, preferably the average fineness is about 3.0 deniers or less, or about 2.5 deniers or less, or about 2.0 deniers or less, or about 1.5 deniers or less.

The ratio of the average fineness of the fiber in the loop layer to the average fineness of the fiber in the base material layer [average fineness of the fiber in the loop layer]/[average fineness of the fiber in the base material layer] is about 1.5 or more and about 30 or less. This ratio is about 1.5 or more, and preferably about 1.7 or more, or about 2 or more, from the point of view of achieving both engagement strength of the loop layer and printing properties of the base material layer. Also this ratio is about 30 or less or preferably about 18 or less, or about 6 or less from the point of view of maintaining the pliability of the loop member, maintaining the mechanical strength of the base material layer, ease of manufacture, and the like.

The above ratio is calculated from the values of the average fineness of the loop layer and the base material layer measured with the fineness measuring instrument Vibromat ME (manufactured by Textechno) or an equivalent measuring instrument. Specifically, first about 10 fibers are sampled as randomly as possible. In this case, fiber that has been damaged, such as cut fiber and the like, cannot be used for measurement, so it is not sampled. Of the sampled fibers, the end of one fiber is held in a tweezers, and the two ends of the fiber are secured by the clamps of the measuring instrument, without twisting or extending the fiber. In this case, the fiber is disposed vertically. The fixed rate of vibration is measured from the vibration of the fiber fixed in the clamps under a certain tension and fiber length, from which the fineness is calculated. This operation is repeated five times, and the average fineness value for the five fibers is taken to be the average fineness. The measurement environment is set to a temperature of 21°C ±1°C, and a humidity of 65% ±2%. From the average fineness obtained for the loop layer and the base material layer, the ratio [average fineness of the fiber in the loop layer]/[average fineness of the fiber in the base material layer] referred to above is calculated.

The short fiber nonwoven fabric included in both the loop layer and the base material layer may each be short fiber nonwoven fabric manufactured using a commonly used method as the method of manufacturing, such as for example carded nonwoven fabric, air-laid nonwoven fabric, and the like. Here, if long fiber nonwoven fabric manufactured by the spunbond method or the melt blown method is used as the base material layer, it will be necessary to use high density nonwoven fabric in order to reduce the air permeability of the base material layer obtained. Also, if the base material layer constituted from the long fiber nonwoven fabric is made thinner using the calendering, it is found that the base material layer obtained becomes stiffer the smaller the thickness. On the other hand, if the base material layer that includes short fiber nonwoven fabric is made thinner using the calendering, pliability and a high level of air permeability can be easily imparted. The method of bonding the fibers in the short fiber nonwoven fabric may be thermal bonding, chemical bonding, hydroentanglement, needle punching, stitch bonding, steam jetting, and the like. In a preferred aspect, the short fiber nonwoven fabric included in the base material layer is thermal bonded nonwoven fabric, from the point of view of obtaining a thin nonwoven fabric with excellent pliability. In a preferred aspect, the short fiber nonwoven fabric included in the loop layer is obtained by fusion bonding the short fiber nonwoven fabric by the high temperature air-through process.

In the fusion bonded short fiber nonwoven fabric included in the loop layer, the fibers from which the short fiber nonwoven fabric is constituted are joined together at fixing sites by fusion of the fibers (typically fusion of the surface of the fiber). In this way, the short fiber nonwoven fabric of the loop layer has excellent mechanical strength, and therefore exhibits good durability of engagement strength under repeated fastening and unfastening.

The fusion bonding can be implemented using any device capable of carrying out the high temperature air-through process. For example, an oven or the like used for the manufacture of nonwoven fabric can be used as the device. However, in a typical aspect of the present disclosure, the fusion bonding is carried out at a higher temperature than the normal temperature conditions for manufacturing nonwoven fabric with their respective materials. Therefore, in a typical aspect of the present disclosure, for example, a device capable of carrying out the air-through process at the temperature described later is used.

When fusion bonding the short fiber nonwoven fabric with a predetermined material, the higher level of fusion of the fibers produced by using a high fusion temperature contributes to increasing the fixing sites between fibers formed by fusion of the fiber surface. When the number of fixing sites between fibers is increased, the gaps between fibers in the short fiber nonwoven fabric are reduced, and the volume of the short fiber nonwoven fabric is reduced. In a typical aspect, the fusion temperature when carrying out the fusion by the high temperature air-through process (specifically, the air temperature) and the air blow rate can be designed in accordance with the desired extent of formation of the fixing sites in accordance with the purpose. The following is a description of an aspect exemplifying the temperature and air blow rate, but the present disclosure is not limited thereto.

In a preferred aspect in the case that the sheath is polyethylene, the short fiber nonwoven fabric of the loop layer is fused at a fusion temperature (for example, the air temperature of the high temperature air-through process) of from about 135°C to about 160°C. From the point of view of preventing drop out of fibers of the short fiber nonwoven fabric in the loop layer by forming the fixing sites well, and obtaining good mechanical strength and therefore good durability of engagement strength, the fusion temperature is about 135°C or higher, or about 140°C or higher. From the point of view of maintaining good pliability and air permeability of the loop layer, the fusion temperature is about 160°C or less, or about 150°C or less, or about 145°C or less.

In a preferred aspect, from the point of view of forming the fixing sites well, the difference (T1-T2) between the fusion temperature (T1) and the melting point (T2) of the material from which the surface of the fiber to be pressure bonded is about 5°C or more, or about 10°C or more, or about 30°C or more.

From the point of view of preventing drop out of fibers of the short fiber nonwoven fabric in the loop layer by forming the fixing sites well, and obtaining good mechanical strength and therefore good durability of engagement strength, the air blow rate in the high temperature air-through process is about 1% or more, or about 10% or more, or about 20% or more, or about 30% or more, and from the point of view of preventing too many fixing sites and maintaining good pliability and air permeability, the air blow rate in the high temperature air-through process is about 100% or less, or about 50% or less. Note that the air blow rate is selected in a balanced manner with the temperature.

In a preferred aspect, the tensile strength at break of the loop layer is about 20 N/50 mm or more and about 200 N/50 mm or less. In a preferred aspect, from the point of view of obtaining good engagement strength of the loop member, the tensile strength is about 20 N/50 mm or more, or about 25 N/50 mm or more, or about 30 N/50 mm or more, and from the point of view of obtaining good pliability and air permeability in the loop member is about 200 N/50 mm or less, or about 100 N/50 mm or less.

In a typical aspect, a calendering is substantially not carried out with the object of surface smoothness of the loop layer. In this way, the short fiber nonwoven fabric included in the loop layer can be made to function well as an engaging element. Note that when for example joining and securing the loop layer and the base material layer, subjecting the loop layer to compression, such as compression by a roll or the like, is not eliminated. For example, if surface smoothing is carried out on only one surface of the short fiber nonwoven fabric layer, a portion of the other surface of the short fiber nonwoven fabric layer may also be subjected to surface smoothing at the same time. In this case, there is a possibility that the engagement strength (for example, the peeling strength and the shear strength) of the short fiber nonwoven fabric on the other surface will be reduced. Therefore, in the loop member of the present disclosure, the loop layer is combined with the base material layer that has already been subjected to the calendering, so the loop layer is not subjected to the effect of the calendering on the base material layer, and therefore the loop layer can be formed without damaging the required engagement strength.

The method and the conditions of the calendering to obtain the calendered short fiber nonwoven fabric included in the base material layer can be set in accordance with the purpose. By increasing the density of the base material layer by the calendering, the base material layer can be given a smooth surface.

For example, the calendering is carried out under conditions set so that the short fiber nonwoven fabric of the base material layer is compressed to the required thickness. In an exemplary aspect, if the base material layer is constituted from polypropylene / polyethylene core-in-sheath fiber, the calendering can be carried out under roll temperature conditions of about from 100°C to about 180°C.

The short fiber nonwoven fabric of the calendered base material layer is advantageous in terms of a stable bond between the base material layer and the loop layer, in other words, contributing to stably maintaining the loop layer by the base material layer, and increasing the engagement strength of the loop member. Also, the calendered base material layer can have lower air permeability compared with, for example, nonwoven fabric that has not been calendered, so it is possible to avoid an excessively large air permeability which would become a problem in the manufacturing process, while maintaining the required air permeability by contributing to the use of the nonwoven fabric.

In a typical aspect, the base material layer is calendered to the extent that is in film form (in other words, the surface of the nonwoven fabric is highly smooth, and in a form that fine printing can be carried out on the surface of the nonwoven fabric). The air permeability of the base material layer after being calendered into film form is lower compared with the base material layer prior to the calendering.

In a preferred aspect, the thickness of the loop layer is about 0.5 mm or more and about 20 mm or less. From the point of view of maintaining good mechanical strength and obtaining good engagement strength and durability thereof under repeated fastening and unfastening, preferably the thickness of the loop layer is about 0.5 mm or more, or about 1.0 mm or more, or about 1.5 mm or more. From the point of view of low cost and good pliability, preferably the thickness of the loop layer is about 20 mm or less, or about 10 mm or less, or about 2.0 mm or less.

In one aspect of the present invention, the thickness of the base material layer is about 15 µm or more and about 100 µm or less. From the point of view of maintaining good mechanical strength and obtaining good engagement strength, the thickness of the base material layer is about 15 µm or more, and preferably is about 20 µm or more, or about 35 µm or more. From the point of view of low cost and good pliability, the thickness is about 100 µm or less, and preferably about 85 µm or less, or about 70 µm or less, or about 55 µm or less. In the base material layer constituted from short fiber nonwoven fabric (for example, thermal bonded nonwoven fabric), when the thickness prescribed above has been achieved by the calendering, it is possible to achieve both reduction of the air permeability down to the required level and maintenance of pliability.

In the present disclosure, the thickness of the loop layer and the base material layer are measured as follows. First, a sample for measurement of thickness with a 10×10 mm area is extracted from the loop member. Next, to measure the loop layer, the base material layer is removed from the measurement sample, and the thickness of the loop layer is measured in the state that it is not joined or secured to the base material layer. Then, to measure the base material layer, the loop layer is removed from the measurement sample, and the thickness of the base material layer is measured in the state that it is not joined or secured to the loop layer. The thickness measurement described above is repeated five times at different locations on the sample, and the average value of the thickness from the results of the five measurements is taken to be the thickness of the loop layer or the base material layer. The thickness measurement is carried out using a thickness measurement instrument (Mitsutoyo Absokute (KK-547-055, or an equivalent instrument), the sample is sandwiched between the cylinder end surface and the base of the measurement instrument, and the thickness of the loop layer or the base material layer is measured by reading the thickness displayed on the digital indicator after two seconds.

In a preferred aspect, the basis weight of the loop layer is about 12 gsm or more and about 50 gsm or less. From the point of view of maintaining the mechanical strength and obtaining good engagement strength and durability thereof under repeated fastening and unfastening, preferably the basis weight is about 12 gsm or more, or about 15 gsm or more, or about 20 gsm or more, or about 25 gsm or more. From the point of view of obtaining the thin loop member with good pliability at low cost, preferably the basis weight is about 50 gsm or less, or about 45 gsm or less, or about 35 gsm or less.

In a preferred aspect, the basis weight of the base material layer is about 8 gsm or more and about 30 gsm or less. From the point of view of maintaining the mechanical strength of the base material layer, preferably the basis weight is about 8 gsm or more, or about 10 gsm or more, or about 12 gsm or more. From the point of view of obtaining the thin loop member with good pliability at low cost, preferably the basis weight is about 30 gsm or less, or about 25 gsm or less, or about 21 gsm or less, or about 18 gsm or less.

A surface treatment (for example, a corona discharge process, an E-beam process) may be carried out on the surface of the printed layer forming surface of the base material layer. Also, a process may be carried out to apply a color to the loop layer and/or the base material layer.

The loop layer and/or the base material layer can typically be made from short fiber nonwoven fabric from the point of view of obtaining the good advantages of the loop member of the present disclosure. Also, an additional layer other than short fiber nonwoven fabric may be included. The loop layer and the base material layer and the short fiber nonwoven fabric included in the loop layer and the base material layer may each be single layer or a plurality of layers. An adhesive layer, a resin film, a knitted fabric, a woven fabric, paper, a laminate of these, and the like can be used as the additional layer. There is no particular limitation on the method of forming the additional layer, and conventional commonly known methods can be used, such as coating, dry lamination, extrusion lamination, wet lamination, thermal lamination, ultrasonics, and the like.

In a typical aspect, the loop layer further includes a printed layer. The printed layer may be directly secured to the base material layer. In the present disclosure, directly securing the printed layer to the base material layer means disposing the printed layer on the base material layer without another member or layer therebetween (in other words, in contact with the base material layer), and, the printed layer substantially cannot be peeled from the base material layer while maintaining its form. Such a printed layer is advantageous in that it enables a thin loop member to be obtained by a simple process.

The printed layer has one or a plurality of layers, and includes at least an ink layer. The printed layer may be constituted from an ink layer only, and may include a base coat and/or a top coat in addition to the ink layer. The base coat and the top coat contribute to improving the adhesion of the ink layer to the base material layer.

The ink layer and the optional base coat and top coat may be continuous layers on the base material layer, or they may be disposed discontinuously, and can be appropriately designed in accordance with the required purpose, for example a design in accordance with the purpose of the ink layer. The design can be selected as desired, such as characters, pictures, patterns, and the like.

The material of the ink layer can be various types of conventionally known inks, and water soluble or solvent type inks can be used. Conventional commonly used resins can be used as the resin included in the ink. For example, acrylic resin, polyurethane resin, polyamide resin, urea resin, polyester resin, vinyl chloride resin, vinyl chloride - vinyl acetate copolymer resin, ethylene - vinyl acetate copolymer resin, olefin resin, chlorinated olefin resin, epoxy resin, oil-based resin, cellulose derivative resin, and the like can be used. With an ink layer with excellent toughness, it is difficult for the ink layer to drop off, even if the ink layer is exposed during use of the article having the loop member according to the present disclosure. From this point of view, an acrylic ink, a urethane ink, or the like are ideal.

Preferably, the ink layer itself has adhesion, from the point of view of fixity of the printed layer on the base material layer. The material used in the adhesive layer referred to above mixed with the ink can be used as the material for forming the ink layer having adhesion.

The thickness of each of the ink layer and the optional base coat and top coat constituting the printed layer can be about 0.5 µm or more and about 20 µm or less, or about 1 µm or more and about 15 µm or less, or about 2 µm or more and about 10 µm or less, from the point of view of toughness of the printed layer and the wearing feeling (pliability, air permeability, and the like), although this is not a limitation.

In one aspect, the printed layer may be bonded to the base material layer by adhesive. In this case, the fixity of the printed layer is good. Adhesive materials can include tacky adhesive polymer such as acrylic polymer (for example, SK-Dyne, an acrylic pressure sensitive adhesive that can be commercially obtained from Soken Chemical & Engineering Co., Ltd.), silicone polymer, rubber-based polymer, and the like, or a hot melt type adhesive such as for example Jet-melt™ EC-3748 (commercially available from 3M Japan), and the like. A tackifying resin, a crosslinking agent, or other additives may be optionally combined with the tacky adhesive polymer.

The thickness of the adhesive can normally be from about 5 µm to about 200 µm. The adhesive can be formed by, for example, applying adhesive material such as those described above onto the surface of the base material layer, and drying it.

The loop member of the present disclosure can be manufactured by various methods. In an exemplary aspect, the loop member can be manufactured by a method that includes: preparing short fiber nonwoven fabric for the loop layer and the short fiber nonwoven fabric for the base material layer; performing a calendering on the short fiber nonwoven fabric for the base material layer; fusion bonding the short fiber nonwoven fabric for the loop layer; laminating the calendered short fiber nonwoven fabric and the fusion bonded short fiber nonwoven fabric for the loop layer, and joining them together to obtain a laminated web that includes the base material layer and the loop layer; and optionally forming the printed layer on the base material layer side of the laminated web.

The manufacture of the short fiber nonwoven fabric, the calendering on the base material layer, and the fusion bonding of the loop layer can, for example, be carried out by the methods and under the conditions as described previously. Next, the calendered short fiber nonwoven fabric and the fusion bonded short fiber nonwoven fabric for the loop layer are laminated.

In a typical aspect, the loop layer and the base material layer are joined together by emboss finishing, chemical bonding, water jetting, air-through (including high temperature air-through), or the like. FIG. 2 illustrates an example of a loop member according to one aspect of the present invention, showing the loop layer and the base material layer secured by embossing. As illustrated in FIG. 2, in the loop member 1, the base material layer 11 and the loop layer 12 can be joined together by an embossed pattern A. Various embossed pattern shapes can be formed by emboss finishing, for example, a rectangle, a wave form, and the like. For example, in an aspect exemplifying a joining region joining the loop layer and the base material layer, if the loop layer and/or the base material layer include carded nonwoven fabric, preferably the pitch of the joining regions in the fiber direction of the carded nonwoven fabric is arranged so that it is shorter than the pitch of the joining regions in the direction substantially normal thereto. Such joining regions are advantageous as it is possible to avoid fluffing of the carded nonwoven fabric. The loop layer is joined to the calendered base material layer, so the loop layer can be stably and strongly secured to the base material layer. Therefore, when the loop member is peeled from a male member or the like, it is difficult for problems such as peeling of the loop layer from the base material layer, tearing of the loop layer, failure, and the like to occur. The emboss finishing can be carried out under conditions of temperature from about 110°C to about 180°C, and pressure in the range from 0 N/m² to about 1,000 N/m².

The method of forming the printed layer on the base material layer can be, for example, a method of directly coating the base material layer with the material for forming the printed layer (in the present disclosure, referred to as the printing materials). Also, a method in which the printed layer that is formed in advance on a liner is transferred onto the printed layer, and the liner removed, or the like, can be used. The transfer method as described above is desirable because it is difficult for the ink of the printed layer to pass through the base material layer and the loop layer.

In the transfer method, specifically first the printed layer is formed on the liner. In order to transfer the printed layer onto the base material layer, preferably the liner has a surface with appropriate releasing properties. Various types of sheet that are conventionally used as liners for transfer can be used as the liner, for example, silicone covered craft paper, silicone covered polyethylene covered paper, silicone covered or uncovered polymer material (for example, polyethylene, polypropylene, and the like), or a base material covered with a polymer releasing agent, for example, silicone urea, urethanes, long chain alkyl acrylate, and the like. Suitable commercial release liners include that which is sold under the commercial name of "POLYSLIC" from Rexam Release of Oakbrook, Illinois, and that which is sold under the commercial name of "EXHERE" from P. H. Glatfelter Company of Spring Grove, Pennsylvania. For example, an emboss finishing or the like may be carried out on the liner on the printed layer forming surface.

The printing materials are applied to such a liner. In a typical aspect, the ink is applied to the liner by any printing method such as for example roll application, gravure application, curtain application, spray application, screen printing, and the like. Or, for example, a top coat, the ink, and a base coat may be applied to the liner in that order. By the above procedures, a transfer sheet in which the printed layer is formed on the liner is obtained.

Next, the printed layer is transferred from the liner to the base material layer by passing the transfer sheet and the laminated web between a pair of rollers, so that the printed layer side of the transfer sheet and the base material layer side of the laminated web are brought into opposition to each other. In this way, the loop member with the printed layer formed on the base material layer can be obtained.

Note that when the printed layer has the ink layer, a base coat, and/or a top coat, the printed layer may be formed sequentially by a plurality of processes. For example, in the case of a printed layer made from a base coat, an ink coat, and a top coat, first the base coat is formed on the base material layer, next the ink layer is transferred, and next the top coat may be formed. By the method described above, the printed layer can be directly secured to the base material layer.

In a preferred aspect, the basis weight of the loop member is about 20 gsm or more and about 60 gsm or less. From the point of view of maintaining the mechanical strength and obtaining good engagement strength of the loop member, preferably the basis weight is about 20 gsm or more, or about 25 gsm or more, or about 28 gsm or more, or about 33 gsm or more. From the point of view of obtaining a thin loop member with good pliability at low cost, preferably the basis weight is about 60 gsm or less, or about 50 gsm or less, or about 43 gsm or less, or about 37 gsm or less.

In a preferred aspect, the 90 degree peeling strength between the loop member and another fastening member (specifically hooks for a surface fastener) that is engaged thereto is about 0.2 N/25.4 mm or more and about 10 N/25.4 mm or less. The above 90 degree peeling strength is measured using a 248 pin per square centimeter (1600 pin per square inch) hook member (model 1600DH manufactured by 3M Company) in accordance with JTM-1221. From the point of view of good engagement strength, preferably the 90 degree peeling strength is about 0.2 N/25.4 mm or more, or about 0.3 N/25.4 mm or more, or about 0.4 N/25.4 mm or more, or about 0.45 N/25.4 mm or more. From the point of view of feeling during use, preferably the 90 degree peeling strength is about 10 N/25.4 mm or less, or about 8 N/25.4 mm or less, or about 7 N/25.4 mm or less, or about 6 N/25.4 mm or less.

In a preferred aspect, between the loop member and another fastening member (specifically hooks for a surface fastener) that is engaged thereto when fastening and peeling at 90 degrees is carried out 20 times, the 90 degree peeling strength on the 20th time is about 0.1 N/25.4 mm or more and about 5.0 N/25.4 mm or less. The above 90 degree peeling strength is measured using a 248 pin per square centimeter (1600 pin per square inch) hook member (model 1600DH manufactured by 3M Company) in accordance with JTM-1221. From the point of view of good engagement strength, preferably the 90 degree strength is about 0.1 N/25.4 mm or more, or about 0.2 N/25.4 mm or more, or about 0.3 N/25.4 mm or more, or about 0.4 N/25.4 mm or more. From the point of view of feeling during use, preferably the 90 degree peeling strength is about 5.0 N/25.4 mm or less, or about 3.0 N/25.4 mm or less, or about 1.0 N/25.4 mm or less.

In a preferred aspect, the shear strength between the loop member and another fastening member (specifically hooks for a surface fastener) that is engaged thereto is about 25 N/20 mm × 25.4 mm or more. The above shear strength is measured using a 248 pin per square centimeter (1600 pin per square inch) hook member (model 1600DH manufactured by 3M Company) in accordance with JTM-1235. From the point of view of good engagement strength, preferably the shear strength is about 25 N/20 mm × 25.4 mm or more, or about 30 N/20 mm × 25.4 mm or more. There is no particular upper limit on the shear strength, but from the point of view of ease of manufacture and strength of the fastening member, it may be, for example, about 100 N/20 mm × 25.4 mm or less.

In a preferred aspect, the shear strength after 20 repetitions of fastening and 90 degree peeling between the loop member and another fastening member (specifically hooks for a surface fastener) that is engaged thereto in accordance with JTM-1221 is about 5 N/20 mm × 25.4 mm or more and about 100 N/20 mm × 25.4 mm or less. The above shear strength is measured using a 248 pin per square centimeter (1600 pin per square inch) hook member (model 1600DH manufactured by 3M Company) in accordance with JTM-1235. From the point of view of good engagement strength, preferably the shear strength is about 5 N/20 mm × 25.4 mm or more, or about 9 N/20 × 25.4 mm or more, or about 14 N/20 mm × 25.4 mm or more. There is no particular upper limit on the shear strength, but from the point of view of ease of manufacture and strength of the fastening member, it may be, for example, about 100 N/20 mm × 25.4 mm or less.

In a preferred aspect, the tensile strength of the loop member when extended by 5% is controlled to be within a prescribed range in accordance with the purpose. If the tensile strength of the loop member is too high, the loop member tends to be too hard. On the other hand, if the tensile strength of the loop member is too low, there is a possibility of occurrence of the problem that the loop member is extended in the MD direction during manufacture of a sanitary article (diaper or the like), or the problem that when a sanitary article (diaper or the like) having the loop member is being used, the loop layer is extended due to shear from the hooks combined with the loop member (when the tensile strength in the CD direction is too low). Note that in the present disclosure, the MD direction of the loop member means the machine direction during manufacture of the loop member. The MD direction of the loop member during manufacture normally coincides with the MD direction of the loop layer and base material layer during manufacture. Also, the CD direction means the direction normal to (in other words, at 90 degrees to) the MD direction. From the above point of view in the MD direction, preferably the tensile strength can be about 7 N/25.4 mm or more, or about 10 N/25.4 mm or more, or about 12 N/25.4 mm or more, and preferably about 200 N/25.4 mm or less, or about 100 N/25.4 mm or less, or about 50 N/25.4 mm or less. In the CD direction, preferably the tensile strength can be about 2.5 N/25.4 mm or more, or about 3 N/25.4 mm or more, or about 3.5 N/25.4 mm or more, and preferably about 50 N/25.4 mm or less, or about 30 N/25.4 mm or less, or about 20 N/25.4 mm or less.

The loop member of the present disclosure can be used for securing items, such as for example flooring materials, wall materials, clothing, cleaning members, automobile interior materials, and the like. As a result of its constitution, the loop member of the present disclosure has good pliability and air permeability, and good engagement strength and durability thereof when repeatedly fastened and unfastened, so it is ideal as the loop member for a surface fastener fitted to a sanitary article, in particular an adult diaper.

Another aspect of the present invention provides an adult diaper that includes a surface fastener that includes the loop member according to an aspect of the present invention as described above.

Examples of sanitary articles include diapers for children and adults, napkins for sanitary and other uses, and the like, but the loop member of the present disclosure has good durability of engagement strength under repeated fastening and unfastening, so it is particularly ideal for application to adult diapers where such repeated fastening and unfastening frequently occurs. In a typical aspect, the loop member of the present disclosure can be used as a surface fastener for sanitary articles, in particular adult diapers, in combination with the loop member of the present disclosure or any other fastening member.

In a preferred aspect, the sanitary article has excellent air permeability. More specifically, from the point of view of being able to impart a good wearing feeling to a sanitary article, preferably the air permeance of the sanitary article measured by the Gurley method is about 5 seconds or less. More preferably, the value is about 3 seconds or less, and still more preferably is about 1 second or less. There is no lower limit in particular, but in one aspect, it is about 0.1 seconds or higher.

There is no particular limitation on the method of manufacturing the sanitary article, but for example the following method can be used. For the elements of the sanitary article apart from the loop member, conventional commonly known elements can be adopted as desired, and here they are not described in detail. In the sanitary article, any conventional commonly known method can be used as the method of fitting the loop member to the object to which it is to be applied. The surface of the loop member on which the printed layer is formed is joined to the object to which it is to be applied by a conventional commonly known method (glue, thermal bonding, adhesion by ultrasonic processing or the like, stitching, mechanical fixing using a stapler, and the like). For securing by glue, a commonly known pressure-sensitive adhesive such as a rubber-based type such as SIS, SBS, or the like, an acrylic-based type, an EVA type, and the like can be selected as appropriate as necessary, but there is no limitation to these resins.

### EXAMPLES

The present invention will be explained in further detail below based on working examples, but the present invention is not limited to the following working examples.

### <Manufacture of the Loop Member>

### Working Examples 1 through 7 and Comparative Example 1

### (Short Fiber Nonwoven Fabric for the Loop Layer)

The following carding nonwoven fabrics were used. The melting point of the sheath was about 115°C, and the melting point of the core was about 163°C.

Product Number: 6.6 ESC cure repeat PE 1185, polyethylene (sheath) / polypropylene (core) two component fiber, average fineness: 6 deniers, fiber length: 40 mm, commercially available from Fibervisions Corporation

Product Number: SESC4013, polyethylene (sheath) / polypropylene (core) two component fiber, average fineness: 4 deniers, fiber length: 40 mm, commercially available from Fibervisions Corporation Product Number: ESC225SDGK, average fineness: 2 deniers, polyethylene (sheath) / polypropylene (core) two component fiber, fiber length: 40 mm, commercially available from Fibervisions Corporation

Product Number: ETC212C, average fineness: 12 deniers, polyethylene (sheath) / polypropylene (core) two component fiber, fiber length: 40 mm, commercially available from Fibervisions Corporation

### (Fusion Bonding the Loop Layer)

The short fiber nonwoven fabric was fusion bonded by high temperature air-through processing in the following oven under the following conditions, to obtain the short fiber nonwoven fabric for the loop layer.
Oven: STRAHM HiPer (TM) Therm System (manufactured by Strahm Textile Systems AG)
Line speed: As shown in Table 1 and Table 2
Air-through temperature: As shown in Table 1 and Table 2
Air blow rate(*): As shown in Table 1 and Table 2
(*) Percentage of the oven maximum flow rate as 100%

Also, carding nonwoven fabric (Product Name: ESC cure repeat PE 1185 or SESC4014, average fineness: 1.5 deniers, fiber length: 40 mm, commercially available from Fibervisions Corporation) was passed between heated rollers at 150°C and 100% calendered (with a football pattern), and short fiber nonwoven fabric (basis weight: 15 gsm, fineness: 1.5 deniers) for the base material layer was obtained. The short fiber nonwoven fabric for the loop layer and the short fiber nonwoven fabric for the base material layer obtained as described above were overlaid, and laminated by pattern emboss finishing at a temperature of about 135°C and a nip pressure of 80 kg.

### Comparative Example 2

KLL GKL: Product Number: CLP-06603, commercially available from 3M Company.

### <Property Evaluation>

### 1. 90° Peeling Strength

The 90 degree peeling strength was measured using a 248 pin per square centimeter (1600 pin per square inch) hook member (model 1600DH manufactured by 3M Company) in accordance with JTM-1221. The loop member and the male member were joined and peeled at 90 degrees 20 times, and the first and 20th 90 degree peeling strength were recorded.

### 2. Shear Strength

The shear strength was measured using a 248 pin per square centimeter (1600 pin per square) inch hook member (model 1600DH manufactured by 3M Company) in accordance with JTM-1235. The shear strength measured after engaging the loop member and the male member was taken to be the first shear strength. Then, the loop member and the male member were fastened and peeled at 90 degrees 20 times, then the loop member and the male member were fastened and the shear strength was measured, and this was taken to be the 20th shear strength.

### 3. Tensile Strength

The tensile strength was measured by the following method using a Tensilon universal testing machine (model RTG-1225, manufactured by A&D Company, Ltd.).

The loop layer was cut with a leather cutter to produce a sample of length 100 mm or more and width 50 mm.

The Tensilon settings were as follows.
Zipper spacing: 100 mm
Tension speed: 300 mm/minute

The sample was attached to the zipper, and the tensile strength at break was measured.

### 4. Surface Condition of the Loop Layer

The surface condition of the loop layer of the loop members manufactured for Working Example 1 and Comparative Example 1 was observed using an optical microscope. FIG. 3 illustrates an image of the surface of the loop layer in Working Example 1, and FIG. 4 illustrates an image of the surface of the loop layer in Comparative Example 1. FIGS. 3 and 4 were taken with a magnification of 175.

**Table 1**

| | | | Working Example 1 | Working Example 2 | Working Example 3 | Working Example 4 | Comparati ve Example 1 | Comparati ve Example 2 |
|---|---|---|---|---|---|---|---|---|
| Loop layer | Fineness (deniers) | | 6 | 4 | 2 | 12 | 4 | - |
| | Fiber material | | PE/PP (Sheath/co re) | PE/PP (Sheath/co re) | PE/PP (Sheath/co re) | PE/PET (Sheath/co re) | PE/PP (Sheath/co re) | PET (KLL) |
| | Basis weight (gsm) | | 30 | 30 | 30 | 30 | 30 | - |
| | Line speed (mpm) | | 60 | 60 | 60 | 60 | 60 | - |
| | Air-through temperature (°C) | | 142 | 142 | 142 | 142 | 131 | - |
| | Air blow rate (%) | | 30 | 30 | 30 | 30 | 23 | - |
| | Tensile Strength at Break (N/50 mm) | | 31 | 42 | NA | 21 | 20 | - |
| | Thickness (mm) | | 1.38 | 1.03 | NA | 1.6 | 1.27 | - |
| Base material layer | Fineness (deniers) | | 1.5 | 1.5 | 1.5 | 1.5 | 1.5 | - |
| | Fiber material | | PE/PP | PE/PP | PE/PP | PE/PP | PE/PP | - |
| | Basis weight (gsm) | | 15 | 15 | 15 | 15 | 15 | - |
| Evaluation | Peeling Strength (JTM1221) (N/25.4 mm) | 1st time | 3.0 | 2.5 | 0.6 | 2.5 | 3.7 | 2.0 |
| | | 20^{th} time | 0.5 | 0.45 | 0.47 | 0.2 | NA | 0.45 |
| | Shear Strength (JTM1235) (N/20 mm×25.4 mm) | 1st time | 48 | 42 | 39 | 35 | 45 | 48 |
| | | 20^{th} time | 15 | 16 | 14 | 9 | 0 | 17 |

**Table 2**

| | | | Working Example 5 | Working Example 6 | Working Example 7 |
|---|---|---|---|---|---|
| Loop layer | Fineness (deniers) | | 6 | 4 | 2 |
| | Fiber material | | PE/PP (Sheath/core) | PE/PP (Sheath/core) | PE/PP (Sheath/core) |
| | Basis weight (gsm) | | 30 | 30 | 30 |
| | Line speed (mpm) | | 60 | 60 | 60 |
| | Air-through temperature (°C) | | 146 | 146 | 146 |
| | Air blow rate (%) | | 30 | 30 | 30 |
| Base material layer | Fineness (deniers) | | 1.5 | 1.5 | 1.5 |
| | Fiber material | | PE/PP | PE/PP | PE/PP |
| | Basis weight (gsm) | | 15 | 15 | 15 |
| Evaluation | Peeling Strength (JTM1221) (N/25.4 mm) | 1st time | 0.98 | 0.25 | 0.2 |
| | | 20^{th} time | NA | NA | NA |
| | Shear Strength (JTM1235) (N/20 mm×25.4 mm) | 1st time | 32 | 7 | 19 |
| | | 20^{th} time | NA | MA | NA |

The loop member of each working example showed good peeling strength and shear strength. Working Examples 1 to 4 showed good peeling strength and shear strength even after 20 repetitions of fastening and unfastening (in other words, good durability of peeling strength and shear strength). The durability of the peeling strength and shear strength of each working example compares favorably with that of the knit loop of Comparative Example 2. On the other hand, in the case of the loop member of Comparative Example 1, in the peeling test, the loop layer was unable to maintain the weight in 10 to 15 repetitions, and the shear strength dramatically reduced after repeated fastening and unfastening. In Comparative Example 1, the loop layer was formed under low temperature air-through conditions, so the loop layer was not substantially fusion bonded.

### [Field of Industrial Use]

The loop member of the present disclosure can be ideally applied to, for example, sanitary articles, in particular adult diapers.

### [Reference Numerals]

- 1: Loop member
- 11: Base material layer
- 12: Loop layer
- 13: Printed layer

## Claims

1. A loop member for a surface fastener, comprising: a loop layer; and a base material layer,
the loop layer including fusion bonded short fiber nonwoven fabric,
the base material layer including calendered short fiber nonwoven fabric,
the ratio of an average fineness of the fiber in the loop layer to an average fineness of the fiber in the base material layer [average fineness of the fiber in the loop layer] / [average fineness of the fiber in the base material layer] being from 2 to 18, and a thickness of the base material layer being from 15 µm to 100 µm, wherein the short fiber nonwoven fabric of the loop layer includes core-in-sheath fibers that include a polypropylene core with a first melting point, and a polyethylene sheath with a second melting point that is lower than the first melting point, and has an average fineness of 4.0 deniers or greater and 10.0 deniers or less, as measured by an average fineness measurement as described in the description.

2. The loop member according to claim 1, wherein the short fiber nonwoven fabric of the loop layer is fusion bonded at a temperature between the first melting point and the second melting point.

3. The loop member according to claim 1 or 2, wherein the short fiber nonwoven fabric of the loop layer and the short fiber nonwoven fabric of the base material layer each include core-in-sheath fiber that includes a polypropylene core and a polyethylene sheath.

4. The loop member according to claim 3, wherein the short fiber nonwoven fabric of the loop layer is fusion bonded at a temperature from 135°C to 145°C.

5. The loop member according to any one of claims 1 to 4, wherein when fastened to a hook for a surface fastener that includes projections and is capable of being engaged with the loop member, and peeled 20 times, the 90 degree peeling strength of the loop member on the 20th repetition is 0.2 N/25.4 mm or more and 5.0 N/25.4 mm or less, as measured by a 90 degree peeling measurement as described in the description.

6. The loop member according to any one of claims 1 to 5, further comprising a printed layer disposed on the base material layer.

7. An adult diaper comprising the loop member described in any one of Claims 1 to 6.

## Patentansprüche

1. Ein Schlaufenelement für einen Oberflächenverschluss, aufweisend: eine Schlaufenschicht; und eine Grundmaterialschicht,
wobei die Schlaufenschicht einen schmelzgebundenen Kurzfaservliesstoff aufweist,
wobei die Grundmaterialschicht kalandrierten Kurzfaservliesstoff aufweist, wobei das Verhältnis einer mittleren Feinheit der Faser in der Schlaufenschicht zu einer mittleren Feinheit der Faser in der Grundmaterialschicht [mittlere Feinheit der Faser in der Schlaufenschicht] / [mittlere Feinheit der Faser in der Grundmaterialschicht] 2 bis 18 beträgt und eine Dicke der Grundmaterialschicht 15 µm bis 100 µm beträgt, wobei der Kurzfaservliesstoff der Schlaufenschicht Kern-in-Mantel-Fasern enthält, die einen Polypropylenkern mit einem ersten Schmelzpunkt und einen Polyethylenmantel mit einem zweiten Schmelzpunkt, der niedriger als der erste Schmelzpunkt ist, enthalten, und eine durchschnittliche Feinheit von 4,0 Denier oder mehr und 10,0 Denier oder weniger, gemessen durch eine durchschnittliche Feinheitsmessung, wie in der Beschreibung beschrieben, aufweist.

2. Das Schlaufenelement nach Anspruch 1, wobei der Kurzfaservliesstoff der Schlaufenschicht bei einer Temperatur zwischen dem ersten Schmelzpunkt und dem zweiten Schmelzpunkt schmelzgebunden ist.

3. Das Schlaufenelement nach Anspruch 1 oder 2, wobei der Kurzfaservliesstoff der Schlaufenschicht und der Kurzfaservliesstoff der Grundmaterialschicht jeweils eine Kern-in-Mantel-Faser enthalten, die einen Polypropylenkern und einen Polyethylenmantel enthält.

4. Das Schlaufenelement nach Anspruch 3, wobei der Kurzfaservliesstoff der Schlaufenschicht bei einer Temperatur von 135 °C bis 145 °C schmelzgebunden ist.

5. Das Schlaufenelement nach einem der Ansprüche 1 bis 4, wobei, wenn es an einem Haken für einen Oberflächenverschluss befestigt ist, der Vorsprünge aufweist und mit dem Schlaufenelement in Eingriff gebracht und 20 Mal abgezogen werden kann, die 90-Grad-Schälfestigkeit des Schlaufenelements bei der 20. Wiederholung 0,2 N/25,4 mm oder mehr und 5,0 N/25,4 mm oder weniger beträgt, gemessen durch eine 90-Grad-Schälmessung, wie in der Beschreibung beschrieben.

6. Das Schlaufenelement nach einem der Ansprüche 1 bis 5, das ferner eine Druckschicht aufweist, die auf der Grundmaterialschicht vorgesehen ist.

7. Eine Erwachsenenwindel, aufweisend das Schlaufenelement, das in einem der Ansprüche 1 bis 6 beschrieben ist.

## Revendications

1. Élément à boucles pour un élément de fixation de surface, comprenant: une couche de boucles, et une couche de matériau de base,
la couche de boucles incluant un tissu non tissé à fibres courtes lié par fusion,
la couche de matériau de base incluant un tissu non tissé calandré à fibres courtes,
le rapport d'une finesse moyenne de la fibre dans la couche de boucles sur une finesse moyenne de la fibre dans la couche de matériau de base [finesse moyenne de la fibre dans la couche de boucles] / [finesse moyenne de la fibre dans la couche de matériau de base] allant de 2 à 18, et une épaisseur de la couche de matériau de base allant de 15 µm à 100 µm, dans lequel le tissu non tissé à fibres courtes de la couche de boucles inclut des fibres âme-dans-gaine qui incluent une âme en polypropylène avec un premier point de fusion, et une gaine en polyéthylène avec un deuxième point de fusion qui est inférieur au premier point de fusion, et a une finesse moyenne de 4,0 deniers ou plus et de 10,0 deniers ou moins, telle que mesurée par une mesure de finesse moyenne telle que décrite dans la description.

2. Élément à boucles selon la revendication 1, dans lequel le tissu non tissé à fibres courtes de la couche de boucles est lié par fusion à une température entre le premier point de fusion et le deuxième point de fusion.

3. Élément à boucles selon la revendication 1 ou 2, dans lequel le tissu non tissé à fibres courtes de la couche de boucles et le tissu non tissé à fibres courtes de la couche de matériau de base incluent chacun une fibre âme-dans-gaine qui inclut une âme en polypropylène et une gaine en polyéthylène.

4. Élément à boucles selon la revendication 3, dans lequel le tissu non tissé à fibres courtes de la couche de boucles est lié par fusion à une température allant de 135 °C à 145 °C.

5. Élément à boucles selon l'une quelconque des revendications 1 à 4, dans lequel, lorsqu'il est fixé à un crochet pour une fixation de surface qui inclut des saillies et est susceptible d'être en prise avec l'élément à boucles, et pelé 20 fois, la résistance au pelage à 90 degrés de l'élément à boucles sur la 20e répétition est de 0,2 N/25,4 mm ou plus et de 5,0 N/25,4 mm ou moins, telle que mesurée par une mesure de pelage à 90 degrés telle que décrite dans la description.

6. Élément à boucles selon l'une quelconque des revendications 1 à 5, comprenant en outre une couche imprimée disposée sur la couche de matériau de base.

7. Couche pour adulte comprenant l'élément à boucles décrit dans l'une quelconque des revendications 1 à 6.
